

Dec. 14, 1937.

C. H. CAMPBELL

2,102,255

## PROCESS FOR THE MANUFACTURE OF COMPOSITE GLUE PRODUCTS

Filed Nov. 6, 1935



Fig. 1.



Fig. 3.



Fig. 2.

INVENTOR.

CHARLES H. CAMPBELL.

BY

Albert B. Briggs

ATTORNEY.

## UNITED STATES PATENT OFFICE

2,102,255

PROCESS FOR THE MANUFACTURE OF  
COMPOSITE GLUE PRODUCTS

Charles H. Campbell, Kent, Ohio

Application November 6, 1935, Serial No. 48,468

8 Claims. (Cl. 134—46)

This invention relates to processes for the manufacture of a composite glue product comprising an inert, finely divided base which is covered with a glue film, and is particularly directed to processes for the production of a pulverulent product by spraying a glue solution upon a moving mass of heated, inert powder.

It has heretofore been the practice to make composite glue products by incorporating a powdered base material into a glue solution and then drying the mixture. According to one procedure, such a mixture was dried in trays and the dry material ground. This mode of operation was found quite unsatisfactory because the base material separated from the glue, settling to the bottom of the trays. When the material was subsequently ground, the composite product contained a large amount of glue unassociated with the base.

To obviate the difficulties encountered by reason of a separation of glue and base material, another procedure was developed according to which a mixture of glue with base was agitated during the drying period. While the composite product produced employing this method has a relatively uniform distribution of base in the glue, it has many hard lumps of base particles agglomerated with glue.

These processes for the production of composite glue products require that the mixture of glue and base be heated for a considerable time at a relatively high temperature so that a dry product is produced. Heating the glue in this manner impairs its quality, and the glue used for the production of such composite products loses from twenty-five to about thirty-five per cent of its strength.

Composite products produced according to the foregoing processes, moreover, are very difficult to grind to the fineness necessary in order that the glue in the finished product will be soluble without an undue delay in soaking, swelling, gelling, and dissolving. To grind the products, it is necessary that they be dried to a friable condition. After a short period of grinding, the hygroscopic products, resulting from hydrolysis of the glue on heating, absorb moisture from the air, and it is necessary to redry the product before the grinding can be continued. A considerable loss of glue strength results both from the heating incident to the grinding operation and from the heating required to redry the product. The grinding of the product, moreover, tends to separate the glue from the inert base.

A mixture of glue solution and base may be

flash dried without substantial loss of glue strength according to the processes of my prior Patent 1,940,486 issued December 19, 1933, and the composite products thus produced are readily soluble.

While the products of my patent aforesaid are of excellent character, the equipment required for entirely satisfactory flash drying procedures involves a greater capital expenditure than the apparatus heretofore employed. The handling of the glue-base magma also requires that the best equipment be used because the magma exercises a considerable abrasive action, and the nozzles and similar devices are subject to considerable wear.

I have found that the difficulties heretofore encountered can be avoided and a product of excellent character produced by spraying a glue solution upon a moving body of finely powdered, inert material. Unlike prior procedures, this does not involve handling of a glue-base magma.

By spraying a glue solution upon an agitated mass of finely divided material, the particles of the base material can be uniformly coated with glue, and a readily soluble, pulverulent, composite glue product of uniform character can readily be produced. This product does not require grinding, of course, and a considerable amount of labor and expense is thus avoided.

The glue solution loses a large amount of its water content during the spraying operation, and very little additional drying is required. If the finely divided base be heated, it supplies the additional heat required to complete the drying of the glue. Accordingly, as soon as the required amount of glue has been applied to the base, the product requires no additional heating to complete its manufacture.

The relatively short time during which the glue is heated does not greatly reduce its strength. The glue in products produced according to this invention ordinarily has a glue strength within about six to eight per cent of the strength of the original glue. While the loss of strength is greater than that produced by the processes of my prior patent aforesaid, it is much smaller than the loss ordinarily produced by other prior art processes, which loss may amount to thirty-five per cent of the original glue strength.

The processes of this invention permit the production of composite glue products of diverse character. This flexibility of operation results from the fact that almost every factor determinative of the product characteristics can easily be controlled at will. The temperature of the

base material, the character of the glue spray, and the distance of the spray nozzle from the base material all influence the drying of the glue solution and the coating of the inert base particles.

The processes of this invention may be better understood by reference to the accompanying drawing wherein:

Figure 1 shows a preferred type of apparatus for the practice of my invention;

Figure 2 illustrates a typical nozzle for spraying glue, and

Figure 3 shows a modified form of apparatus suitable for use with continuous processes.

Referring to Figure 1 in more detail, I designates a mixer which is employed to agitate a mass of finely divided inert base material. This mixer is of a conventional type, and is of the same design as mixers heretofore used for mixing and kneading dough, tar, and the like.

A body of base material in the mixer may be agitated by the arms 2 and 3. These arms 2 and 3 are rotated in opposite directions by conventional gears and a motor, not shown.

In order to control the temperature of the mass of finely divided material, the mixer is provided with a steam jacket 4.

As is indicated in the drawing, a glue solution is sprayed upon the agitated mass of base material by means of a nozzle 5. The construction of a suitable nozzle is more fully illustrated in Figure 2.

I have found that it is necessary to employ a special type of nozzle if the best results are to be obtained. Nozzles of conventional design operate satisfactorily for a time, but, after a short period of operation, they become clogged. This clogging of the nozzles is attributable to the cooling effect of the evaporation of glue solution near the nozzles. The cool zone at the nozzle outlet causes glue to deposit as a heavy glue jelly which, in a short time, seals the small nozzle orifice. When the nozzle becomes clogged, it is necessary to clean it as by dissolving the glue in hot water.

A typical nozzle which will operate continuously is shown in Figure 2. The nozzle 5 is provided with a tube 6 which terminates in a spraying orifice. The pipe 6 carries glue solution, and discharges it in a nebular spray upon the inert base material. The outer casing of the nozzle 5 forms a passage 7 around the pipe 6. Steam, hot air, or hot products of combustion are forced thru the passage 7.

By surrounding the glue spray with a stream of hot gases, cooling of the nozzle orifice is avoided and clogging of the nozzle is prevented. The hot gases, moreover, aid in drying the glue solution, and, by control of the gas temperature and velocity, one may effect a desired rate and manner of drying. More will be said hereinafter regarding this type of control.

While the type of nozzle above described is very satisfactory, it will be understood that I do not intend to be limited thereto. Instead of supplying hot gases to the nozzle, one may blow atmospheric air thru the passage 7 and heat it electrically by means of a suitably insulated coil of resistance wire secured to the nozzle casing.

Other means of providing a heated flow of gas around a glue spray will readily occur to those skilled in the art. It will also be understood that the processes of my invention may even be operated for at least a short period with a conventional, unheated nozzle.

Whatever type of nozzle is employed, it is important that a nebular spray be obtained. If the glue solution be discharged upon the base material as large droplets, the glue will not satisfactorily coat the inert powder. The droplets of glue would be present in the final product as difficultly soluble particles. The glue, then, should be atomized to form what is ordinarily termed a nebular spray, and I prefer to use as fine a spray as may economically be maintained.

The sprayed glue particles tend to flatten and to assume a film-like or plate-like form as they move towards the inert base material. After such a plate of glue strikes the inert particles of base material, it is broken and cut up by the particles, thus coating them with glue. When a weak glue is used, even fairly large drops will flatten out enough to result in a pulverulent, composite product. When a stronger or more concentrated glue is used, smaller droplets should be formed as the more coherent solution does not flatten out to so great an extent.

The orifice of the pipe 6 should be of a more or less rectangular cross-section so that an even distribution of glue may be obtained. The cross-section of the glue spray may also be controlled to some extent, if desired, by the cross-section of the hot gas stream surrounding it. It will be understood, however, that while it is desirable to employ a glue spray more or less rectangular in cross-section, this refinement is not essential to the operation of the processes of my invention.

Considering now a specific process employing an apparatus such as that shown in Figure 1, the mixer was filled with finely divided whiting, and the mixer arms were set in motion. Steam at 80 pounds per square inch pressure was admitted to the steam jacket of the mixer, and the mass of whiting brought to a temperature of about 212° F.

After the whiting was at the desired temperature, the speed of the mixer arms was increased so that the whiting was caused to surge towards the center of the mixer. At this time the mixer arms were rotating at about twenty revolutions per minute.

Hot combustion gases at about 250° F. were admitted thru the passage 7. A glue solution containing one part of high grade, hide glue in three parts of water was admitted to the pipe 6 at a pressure of about one hundred pounds per square inch, and was sprayed upon the agitated mass of whiting.

The nozzle was set at an angle of about 40° to the horizontal, and it was located about eighteen inches from the base material being sprayed. This location of the nozzle had previously been determined by experiment.

After an amount of glue solution equivalent to about one part of dry glue for each two parts of whiting had been sprayed upon the base, the spraying of the glue solution was discontinued, and the pulverulent product was dumped from the mixer. The product thus obtained was in finely divided form, and the whiting was rather uniformly coated with glue. This product is very satisfactory as an ingredient of distemper paints and calcimines.

It will readily be understood that while the specific conditions given above are about optimum for the operation set forth, they may be widely varied without departing from the spirit of my invention.

The rate of rotation of the arms may be wide-

ly varied according to the temperatures selected and the rate at which the glue solution is sprayed. The base material must be moved rapidly enough so that no more than enough glue is applied to 5 a given surface layer of particles. The best speed for the mixer arms can readily be determined for a particular installation by experiment.

It has already been noted that the mixer arms rotate in opposite directions, and, in the above 10 procedure, the arms were rotated so that they came up at the outside of the mixer and went down at the center. This is the manner in which these arms are ordinarily rotated, but they may advantageously be rotated in the opposite directions. It will also be understood that conventional mixers in which one set of arms rotates 15 more rapidly than the other may be used, but this is not particularly desirable. Devices of various types which are provided with means capable of moving a body of finely divided material 20 may obviously be used.

The glue solution used can be made with any grade of hide glue, or bone glue, or mixtures of the same at the option of the user. Or if desired, it is possible to employ a glue liquor that 25 has been passed thru evaporators but has not yet been chilled and dried.

About one part of medium grade glue should be 30 present for each two parts of water, but it may be desired to use more dilute or more concentrated solutions particularly with various grades of glue. Too concentrated a solution should not be used because it is difficult satisfactorily to spray and because it may lose its water too quickly. Too dilute a solution, similarly, is not satisfactory because too large an amount of heat will 35 be required to evaporate the excessive amount of water. As will be noted hereinafter, the concentration of the glue solution should be selected with reference to the character of the glue, the operating temperatures, and the operating conditions. Generally, about one part of glue should 40 be used with each two to five parts of water.

The pressure under which the glue solution is 45 supplied to the nozzle will depend upon the nozzle design, the solution concentration, and the character of the glue. Generally, a pressure of the order of one hundred pounds per square inch is required to obtain a suitable nebular spray as above described.

50 The amount of glue sprayed upon the inert mass can, of course, be selected at will. For the production of a composite product suitable for use in calcimines, it is ordinarily desirable to spray an amount of solution equivalent to about one part of glue to each two to eight parts of whiting or gypsum. These proportions may obviously be varied according to the proposed use 55 of the composite glue product.

To produce a composite product suitable for 60 use in calcimines and the like, other finely divided inert materials such as gypsum, clay, talc, and the like may be used as a base. It may also be found desirable to apply a glue solution to a mixture of inert materials. For instance, I may 65 apply a glue spray according to the processes of my invention to a mixture of finely divided calcimine materials as whiting, gypsum, clay, and a suitable dry aniline color.

70 The temperature of the body of base material is an important factor in the operation of the process above described. It will be evident that the steam temperature and pressure applied to the jacket 4 will be governed by the temperature which it is desired to maintain for the inert ma-

terial. To shorten the time that a batch is in a mixer, it will ordinarily be found desirable to pre-heat the inert material before charging it into the mixer. In this way, the inert base can be more quickly and economically heated, and the 5 output of a mixer will be greater.

The temperature of the gas supplied around the glue conduit 6 is also an important factor, and one which must be correlated with the temperature of the inert base. The position of the 10 nozzle must also be selected with reference to the temperatures. It is to be noted that combustion gases were used in the above process because the glue loses less strength if dried in an inert atmosphere. It is preferred, accordingly, to employ an inert gas when convenient.

The heat supplied by the gases in direct heat exchange relation thereto effects a partial drying of the glue solution, and the gas temperature and volume should be selected with reference to the 20 extent of drying desired.

In the process described above, the gas was at a temperature of 250° F. In the distance between the nozzle and the base material, about eighteen inches, the glue solution lost about sixty 25 per cent of its water. If a higher gas temperature were used, the glue would be dried too much unless a more dilute solution were used or unless the nozzle were positioned nearer to the base material. Similarly, if a lower gas temperature 30 were used, the glue solution would not be adequately dried unless the nozzle were positioned further from the base material, or unless a more concentrated solution were used.

It will be evident, then, that the solution concentration, the nozzle position, and the gas temperature must be correlated to obtain a given amount of drying of the solution prior to its contact with the base material. It has already been indicated that the solution concentration is preferably varied within limits, and it will be understood that the solution must be dilute enough to spray, but must not be so dilute as to require excessive heat to remove the moisture. The nozzle position, similarly, can only be varied within 40 limits because if it is too close, the glue solution 45 would not cover a large enough area of base material, and if it is too far the glue particles would lose their velocity and direction.

The gas temperature should generally be between about two-hundred-and-twenty and two-hundred-and-sixty degrees F. for most operations, tho a much wider range of temperatures may be used by suitable adjustment of other factors. The gas temperature, obviously, should 50 be high enough to prevent clogging of the nozzle.

The amount of water to be removed from the glue by the time that it reaches the base material is subject to considerable variation. The glue must not be too dry when it reaches the 60 base material, or it will not be soft enough properly to coat the base particles.

The base material should ordinarily be at a temperature such as will complete the drying of the glue. If a large volume of hot gas is admitted at 7, very little heating of the particles of base material will be required because the hot gases passing over the surface of the base material will dry the glue even after it is on the particles.

70 The base material should not be heated above about 212 to 220° F. because much higher temperatures may result in a loss of glue strength. As soon as the glue has coated the base material and is dry, further heating at a moderate tem- 75

perature effects only a small loss of glue strength. For this reason, the relatively short period of heating to which the material is subjected in the course of its production does not result in an excessive loss of glue strength.

It will be understood that, preferably, the conditions will be such as to dry the glue enough to prevent agglomeration before substantial agglomeration occurs. Following the teachings of my invention, one skilled in the art will experience little difficulty in adjusting the variables above discussed to produce a pulverulent, composite product. It is important, however, that it be understood that the factors must be correlated.

When glue is flash dried according to the processes of my prior patent aforesaid, the high temperatures cause a puffing of the glue. This puffing is probably attributable to the escape of water as steam. Glue which has been puffed in this manner is somewhat sponge-like in structure and, as so great a surface is accessible to water, it is very easily water-soluble.

While the products as produced above are readily water-soluble, it may be desirable to puff them. This can readily be accomplished by raising the base material to a puffing temperature, but a slight loss of glue strength may result if such temperatures be maintained for too long a period.

Alternatively, the gas admitted at 7 can be raised to a puffing temperature, and the high temperatures will prevail only on the surface of the body of inert material. To avoid overheating of the liquid glue, a separate, high temperature gas nozzle may be provided to supply hot gas to the surface of the body of inert material.

In Figure 3 there is illustrated an apparatus by means of which a composite glue product may continuously be produced in either a puffed or an unpuffed condition.

In Figure 3, the reference character 8 designates a rotatable drum of a type frequently used as a drier. The drum 8 is provided with circumferential bearings 9 which rest upon suitable rollers 10. Thrust rollers, not shown, are provided in conventional manner to prevent endwise movement of the drum. The drum is caused to rotate by a girth gear 11, driven by a pinion 12.

A finely divided inert material is fed from hopper 13 by a conveyor screw 14, and the material is steadily and continuously fed to the upper end of drum 8 thru the axial pipe 15.

The inert base material moves towards the lower end of the drum, and, as it moves, it is sprayed with glue by means of a nozzle 16. A hot gas admitted at 17 acts to dry the glue, and the flow of hot gas to the upper end of the drum, countercurrent to its flow, preheats the base material.

The upper end of the drum 8 may be provided with an opening of variable size for the escape of hot gas. By varying the size of the opening, the rate of gas flow may, in some measure, be controlled.

The composite glue product discharged at the lower end of the drum falls upon a conveyor 18 and is carried to a receptacle 19. A scraper 20 may be provided to remove any of the product which adheres to the conveyor.

The considerations as to the type of spray, the temperatures, etc. are similar to those heretofore discussed. The conditions should, preferably, be so selected that a pulverulent, composite product will continuously be produced.

The nozzle 16, as illustrated, does not carry a

flow of hot gas. Under some conditions of operation, the hot gas from 17 will keep the nozzle 16 warm enough to prevent clogging, but it is preferable to provide means to heat the nozzle. The nozzle may be heated by means of an electric resistance secured thereto, or by a steam jacket, or by other indirect heat exchange means. It is to be noted that in using the device of Figure 1, similarly, the nozzle 2 may be heated in this manner, relying on the heat of the base material or on an additional hot gas nozzle for the heat required to dry the glue.

The gas admitted at 17 may be at about 212° F. if it is desired to produce an unpuffed product. If it is desired to produce a puffed product, the gas should be at a relatively higher temperature, say 400° F. The coated product upon which the gas from 17 is directed would be subjected to a high temperature for only a short period. The gas would then pass on to a direct heat exchange with the glue spray where it would be considerably cooled. The somewhat cooled gas would then continue upwardly and preheat the base material.

If convenient, the hot gas admitted at 17 should be inert. If hot combustion gases are used, for instance, the drying of the glue will be accomplished in an inert atmosphere.

Instead of using separate nozzles 16 and 17, a nozzle such as that shown in Figure 2 may be used.

It will be understood that various types of drums may be used in the practice of the above process. For instance, one may employ a drum of known type which has an outer shell serving as an indirect heat exchange means.

While the above processes offer some advantages, the processes employing a device such as is shown in Figure 1 are preferred because of the smaller equipment costs and because of the positive mixing action.

While the processes of my invention are particularly advantageous in the production of a composite product for use in calcimines, it will be understood that such composite glue products can be used in a number of other ways.

It will also be understood that while the preferred processes of this invention lead to a pulverulent product, the process conditions may be modified so as to produce an agglomerated product. Such processes which lead to an agglomerated product are superior to prior art processes leading to a similar product, but, as such material must be ground, it is very desirable to produce directly a pulverulent, composite glue product.

While I have shown a number of illustrative processes, conditions, and devices, I do not intend to be limited thereby, the scope of my invention appearing in the following claims.

I claim:

1. In a process for the production of a pulverulent, composite glue product, the steps comprising heating a finely divided, inert base, agitating the base with the type of agitation accomplished by mixer arms, during the agitation directing a nebular spray of glue solution upon the surface of the agitated base, and simultaneously directing a flow of hot gas around the glue spray partially to dry the glue before it impacts upon the base material, the total heat being sufficient to dry the glue before substantial agglomeration of base particles occurs.

2. In a process for the production of a pul-

verulent, composite glue product, the steps comprising heating a finely divided, inert calcimine base, agitating the base so that its particles are brought to the surface and then displaced in turn by other particles, during the agitation directing a spray of glue solution upon the surface of the agitated base, and simultaneously directing a flow of hot gas around the glue spray partially to dry the glue before it impacts upon the base material, the total heat being sufficient to dry the glue before substantial agglomeration of base particles occurs.

3. In a process for the production of a pulverulent, composite glue product, the steps comprising heating a finely divided, inert calcimine base to a temperature not substantially higher than about 212° F., agitating the base so that its particles are brought to the surface and then displaced in turn by other particles, directing a nebular spray of glue solution upon the surface of the agitated base, simultaneously directing a flow of hot gas around the glue spray partially to dry the glue before it impacts upon the base material, the total heat being sufficient to dry the glue before substantial agglomeration of base particles occurs.

4. In a process for the production of a pulverulent, composite glue product, the steps comprising heating a finely divided, inert calcimine base, agitating the base so that its particles are brought to the surface and then displaced in turn by other particles, directing a spray of glue solution upon the surface of the agitated base, and directing a flow of hot gas towards the base material, the hot gas partially drying the glue before it impacts upon and coats the particles of base material and the heat which the glue solution gains from the gas plus the heat which it gains from the base material being adequate to dry the glue enough to prevent substantial agglomeration of base particles coated therewith.

5. In a process for the production of a pulverulent composite glue product, the steps comprising heating a finely divided, inert calcimine base, agitating the base so that its particles are brought to the surface and then displaced in turn by other particles, heating a glue solution and directing a spray of the heated solution upon the surface of the agitated base, and directing a flow of hot gas towards the base material, the hot gas partially drying the glue before it impacts upon and coats the particles of base material and the heat which the glue solution has

plus that which it gains from the gas plus that which it gains from the base material being adequate to dry the glue enough to prevent substantial agglomeration of base particles coated therewith.

6. In a process for the production of a pulverulent, composite glue product the steps comprising heating a finely divided inert calcimine base by contacting it directly with a flow of hot gas, agitating the base so that its particles are brought to the surface and then displaced in turn by other particles, directing a spray of glue solution upon the surface of the agitated base and directing a flow of hot gas towards the base material thus partially drying the glue before it impacts upon and coats the base material and the heat which the glue solution thus gains from the gas plus the heat which it gains from the base material being adequate to dry the glue enough to prevent substantial agglomeration of base particles coated therewith.

7. In a process for the production of a pulverulent, composite glue product the steps comprising heating a finely divided inert calcimine base by indirect heat exchange, agitating the base so that its particles are brought to the surface and then displaced in turn by other particles, directing a spray of glue solution upon the surface of the agitated base and directing a flow of hot gas towards the base material thus partially drying the glue before it impacts upon and coats the base material and the heat which the glue solution thus gains from the gas plus the heat which it gains from the base material being adequate to dry the glue enough to prevent substantial agglomeration of base particles coated therewith.

8. In a process for the production of a pulverulent composite glue product, the steps comprising heating a finely divided inert calcimine base, agitating the base so that its particles are brought to the surface and then displaced in turn by other particles, directing a spray of glue solution upon the surface of the agitated base, partially drying the glue in its passage towards the base by contacting it directly with hot gas, the heat which is supplied to the glue solution before it impacts upon the base material plus the heat supplied to the glue by the base material being adequate to dry the glue enough to prevent substantial agglomeration of base particles coated therewith.

CHARLES H. CAMPBELL.